

# United States Patent [19]

Kramp et al.

[11]

4,254,215

[45]

Mar. 3, 1981

[54] **PROCESS FOR THE PREVENTION OF DARKENING AND THE FORMATION OF A SEDIMENT IN PHOTOGRAPHIC DEVELOPER SOLUTIONS**

[75] Inventors: **Ekkehard Kramp; John Lenoir; Max Marthaler**, all of Marly, Switzerland

[73] Assignee: **Ciba-Geigy AG, Basel, Switzerland**

[21] Appl. No.: **24,287**

[22] Filed: **Mar. 26, 1979**

[30] **Foreign Application Priority Data**

Mar. 31, 1978 [CH] Switzerland ..... 3478/78  
Feb. 16, 1979 [CH] Switzerland ..... 1547/79

[51] **Int. Cl.<sup>2</sup> ..... G03C 5/30; G03C 5/38**

[52] **U.S. Cl. ..... 430/419; 430/456;  
430/488**

[58] **Field of Search ..... 96/61 M, 66.5, 66.4,  
96/29 R, 66 R, 61 R, 109, 59, 66.1, 66.2**

[56] **References Cited**

## U.S. PATENT DOCUMENTS

3,607,904 9/1971 Willems ..... 96/109

|           |        |                       |         |
|-----------|--------|-----------------------|---------|
| 3,685,991 | 8/1972 | Grasshoff et al. .... | 92/29 R |
| 3,932,480 | 1/1976 | Grasshoff et al. .... | 96/66.5 |
| 4,141,734 | 2/1979 | Lenoir et al. ....    | 96/61 M |

## FOREIGN PATENT DOCUMENTS

|        |        |                      |        |
|--------|--------|----------------------|--------|
| 604151 | 6/1948 | United Kingdom ..... | 96/109 |
| 997031 | 6/1965 | United Kingdom ..... | 96/107 |

*Primary Examiner*—Mary F. Downey

*Attorney, Agent, or Firm*—Sprung, Felfe, Horn, Lynch & Kramer

[57]

## ABSTRACT

A process is described for the prevention of darkening and the formation of a sediment in photographic developer solutions which contain a silver halide developer, a water-soluble silver halide solvent and organic sulfur compounds. The organic sulfur compounds are a combination of (a) an organic thiol compound or thione compound capable of tautomerism and (b) a Bunte salt which contains groups conferring solubility in water. Developer solutions which contain the indicated combination of sulfur compounds are outstandingly stable.

**21 Claims, No Drawings**

PROCESS FOR THE PREVENTION OF  
DARKENING AND THE FORMATION OF A  
SEDIMENT IN PHOTOGRAPHIC DEVELOPER  
SOLUTIONS

When photographic materials containing silver halide are processed, developing is in the main carried out in an alkaline medium and o- or p-dihydroxybenzenes, aminophenols, diaminobenzenes, pyrazolidinones, reductones or hydroxylamine derivatives are used as developer substances. Usually, the developer solution also contains further additives, such as salts of sulfurous acid for stabilising, anti-fogging agents and buffer substances. Furthermore, it is also known to develop photographic material in certain cases in the presence of silver halide solvents. Such silver halide solvents are, for example, organic compounds of divalent sulfur, such as mercapto compounds, thioethers, thioamides or compounds containing an acid —CH grouping, for example bis-methylsulfonylmethane, and also salts of thiocyanic acid or salts of sulfurous acid in high concentration, but especially salts of thiosulfuric acid.

Developers containing such additives are known as fine-grain developers and in-grain developers. (cf. E. 25 Mutter, "Die Technik der Negativ- und Positivverfahren" ("The Techniques of Negative and Positive Processes"), Springer 1955, page 158 to 159). The developing of latent silver nuclei inside the grains is of particular importance in the case of reversal development processes, in which salts of thiocyanic acid are frequently added to the first developer. Further important embodiments of this type are the monobaths, such as are described, say, in U.S. Patent Specification No. 3,857,710 or by G. Haist in "Monobath Manual", Morgan 1960. A further embodiment of this type is a masking developer for the silver dye-bleach process as described in German Offenlegungsschrift No. 2,547,720.

However, many of these developers have the disadvantage that they more or less rapidly reduce the silver halide dissolved in the form of a complex from the photographic material. As a result of this a turbidity and, after some time, a sediment of silver form in the developer and this sediment can adhere both to the photographic material and to parts of the developing equipment. This formation of a sediment proves particularly disadvantageous in the case of equipment which operates continuously. There has been no lack of attempts to find suitable measures against the formation of a silver sediment.

In German Offenlegungsschrift No. 2,437,353 it is proposed to use derivatives of 1-phenyl-5-mercaptopotetrazole in developer for X-ray film to counter the deposition of silver in developing equipment. In U.S. Patent Specification No. 3,173,789 and in German Auslegeschrift 1,175,077 and German Offenlegungsschrift No. 2,003,414 heterocyclic mercapto compounds, and in German Offenlegungsschrift No. 1,909,743 aliphatic mercaptocarboxylic acids, are described as additives to processing solutions to combat the formation of a silver sediment. In U.S. Patent Specification 3,318,701,  $\alpha$ -liponic acid, and in German Offenlegungsschrift No. 2,040,801 4-acylamino-1,2,3-triazoline-5-thiones, are proposed to counter the formation of a sediment. These substances are usually employed in amounts of between 5 and 5,000 mg per liter of developer solution.

It has been found that the proposed additives can delay the formation of a silver sediment for a certain

period, but they have diverse undesired side effects. Substances which have a good clarity-preserving effect have a considerable influence on the characteristics of the developer. In the case of multi-layer colour materials, in particular the sensitivity of the uppermost layer is reduced. When silver dye-bleach materials are subjected to masking developing, disturbances in the masking effect arise. Other substances are unstable in the developer, lose effectiveness rapidly due to atmospheric oxidation or decompose with the formation of secondary products which are malodorous and/or harmful to health. The practical application of the clarity-preserving substances proposed hitherto is made considerably more difficult and in many cases impossible as a result of all of these disadvantages. Finally, in German Offenlegungsschrift No. 2,640,659 a developing process is described in which specific organic di- or tri-sulfides are used to preserve the clarity of developer solutions.

These di- and tri-sulfides are indeed already very suitable for preserving the clarity of, and for preventing the formation of a silver sediment in, photographic developer solutions, but they have the disadvantage that they are accessible by synthesis only with difficulty and, furthermore, that they have to be employed in relatively large amounts in the developing bath in order to obtain the desired effects.

The object of the present invention is, therefore, to provide a novel process for the prevention of darkening and the formation of a sediment in photographic developer solutions, with which process impairment of photographic developing should be largely excluded.

It has now been found that this object can be achieved if a combination of a mercapto compound and a Bunte salt is added to the developer solutions.

It is true that German Offenlegungsschrift No. 1,768,400 already describes the use of Bunte salts in the photographic field, for example as stabilisers for silver halide emulsions or for stabilising photographic materials which have been developed. In contrast to this, however, the Bunte salts according to the present invention are employed in combination with a mercapto compound in developer solutions and are used for a different purpose.

The present invention relates to a process for the prevention of darkening and the formation of a sediment in photographic developer solutions which contain a compound which develops silver halide, a water-soluble silver halide solvent and organic sulfur compounds, which comprises adding to the developer solution, as organic sulfur compounds, a combination of (a) an organic thiol compound or thione compound which is capable of tautomerism and (b) a Bunte salt containing groups which confer solubility in water.

The thiol compounds or thione compounds capable of tautomerism are compounds of the formulae



or



whilst the Bunte salts have the formula



in which formulae A is a nitrogen atom, a carbon atom bonded via a double bond



$R_2$  is hydrogen, substituted or unsubstituted alkyl, substituted or unsubstituted phenyl or a substituted or unsubstituted, saturated or unsaturated 5-membered or 6-membered heterocyclic radical containing nitrogen, oxygen and/or sulfur atoms and  $R_1$  has the meaning defined for  $R_2$  with the exception of hydrogen, or  $R_1$  and  $R_2$  together with the atoms to which they are bonded form a 4-membered, 5-membered or 6-membered heterocyclic ring, D and E are each a substituted or unsubstituted aliphatic, araliphatic, cycloaliphatic, aromatic or heterocyclic radical and W and Z are each a radical of the formulae



or a polyoxyethylene radical which has 2 to 20 oxyethylene units and can be sulfonated, in which formulae G, X and Y are each hydrogen or are alkyl having 1 to 6 carbon atoms which is substituted by hydroxyl, carboxyl or  $-\text{SO}_3\text{H}$  and Y is also phenyl, phenylsulfonic acid, alkylsulfonyl having 1 to 5 carbon atoms, phenylsulfonyl or tolylsulfonyl, M is a monovalent cation and  $\text{A}_1\Gamma$  is a monovalent anion, and n and m are each an integer from 1 to 4 and r is 1 or 2. If r is 1, the Bunte salts have the formula  $(\text{Z})_m-\text{E}-\text{SSO}_3\text{M}$ , in which the symbols are as defined.

The invention also relates to the developer solution for carrying out the process, the concentrates for preparing the developer solutions, the use of the process when developing photographic black-and-white, reversal, chromogenic, X-ray or silver dye-bleach material 5 and also the use of the combination of components (a) and (b) as the additive which suppresses darkening and the formation of a sediment (silver sediment) in photographic developer solutions.

In the mercapto compounds of the formula (1), D is, 55 for example, a substituted or unsubstituted, saturated or unsaturated aliphatic radical having not more than 40 and preferably not more than 20 carbon atoms, preferred radicals being straight-chain  $-(\text{CH}_2)_x-$ ,  $x=1$  to 40) or branched alkylene and alkylidene having not 60 more than 10 carbon atoms. The alkylene and alkylidene bridge members can, if desired, also be interrupted by  $-\text{O}-$ ,  $-\text{SO}_2-$  or  $-\text{NH}-$  or  $-\text{NR}-$  ( $\text{R}=\text{C}_1-\text{C}_4\text{-alkyl}$ ). In addition to alkyl (formation of the branched radicals), for example alkyl having 1 to 5 65 carbon atoms-methyl, ethyl, n-propyl, n-butyl, n-amyl and isomeric radicals-, substituents can be carboxyl, carboxyalkyl having 1 to 3 carbon atoms in the alkyl

moiety, especially carboxymethyl, hydroxyl, mercapto ( $-\text{SH}$ ) and also hydroxy- or mercapto-alkyl each having, for example, 1 to 3 carbon atoms (hydroxymethyl, hydroxyethyl, hydroxypropyl and the corresponding radicals containing mercapto groups). If the substituents are mercapto or mercaptoalkyl groups, the mercaptans of the formula (1) are dimercaptans or can also be poly-mercaptans.

If the bridge member D is a substituted or unsubstituted aliphatic radical, which likewise can contain not more than 40 carbon atoms, such radicals are, in particular, benzylene or phenylethylene radicals, which can be substituted on the phenyl ring by halogen (fluorine, chlorine or bromine), hydroxyl, amino ( $-\text{NH}_2$ ),  $-\text{SO}_3\text{H}$  or  $-\text{SO}_2\text{NH}_2$ .

The cycloaliphatic radicals are in particular derived from cycloalkyl having 1 to 4 cycloalkyl rings and 5 to 10 carbon atoms and preferably having 5 or 6 carbon atoms. Examples are cyclopentyl, cyclohexyl, norbornyl or 1-adamantyl radicals.

The aromatic radicals are as a rule those which are derived from mononuclear or polynuclear, substituted or unsubstituted aromatic compounds having a total of not more than 40 carbon atoms, but especially those derived from benzene. Phenylene is preferred and this can contain, as substituents, alkyl, for example having 1 to 4 carbon atoms, halogen, for example fluorine, chlorine or bromine, hydroxyl, amino ( $-\text{NH}_2$ ),  $-\text{COOH}$ ,  $-\text{SO}_3\text{H}$  or  $-\text{SO}_2\text{NH}_2$ , alkyl, halogen and amino being preferred.

If the bridge member D is a substituted or unsubstituted heterocyclic radical, these radicals are as a rule saturated or unsaturated 5-membered or 6-membered radicals containing nitrogen, oxygen and/or sulfur atoms, for example pyridyl, pyrimidyl, pyridazyl, pyrazolyl, pyrryl, triazinyl, imidazolyl, the triazolyl and tetrazolyl radicals, the oxazolyl and thiazolyl radicals, furyl or thienyl; further radicals are morpholinyl, imidazolinyl, imidazolidinyl, pyrrolidinyl, pyrrolidinyl, tetrahydrofuryl or piperidinyl.

The radicals can, thus, contain 1 to 4 nitrogen atoms, one oxygen atom and/or one sulfur atom. Examples of fused systems are benzimidazoles, quinoxalines, benzoxazoles and benzthiazoles.

In the mercapto compounds of the formula (1),



—SO<sub>2</sub>M or a polyoxyethylene radical which has 2 to 20 oxyethylene units and can be sulfonated. G, X and Y independently of one another can be hydrogen or substituted alkyl having 1 to 6 carbon atoms, possible substituents being hydroxyl, carboxyl or —SO<sub>3</sub>H; Y can also be phenyl, phenylsulfonic acid



alkylsulfonyl having 1 to 5 carbon atoms in the alkyl moiety ( $\text{CH}_3\text{SO}_2-$ ,  $\text{C}_2\text{H}_5\text{SO}_2-$ ,  $\text{C}_3\text{H}_7\text{SO}_2-$ ,  $\text{i-C}_3\text{H}_7\text{SO}_2-$ ,  $\text{C}_4\text{H}_9\text{SO}_2-$  or  $\text{C}_5\text{H}_{11}\text{SO}_2-$ ), phenylsulfonyl



or tolylsulfonyl



G, X and Y together with the nitrogen atom can, furthermore, also form a saturated or unsaturated 5-membered or 6-membered ring, for example a pyridinium ring. M is a monovalent cation, especially the hydrogen cation ( $\text{H}^{\oplus}$ ), and also an alkali metal cation ( $\text{Na}^{\oplus}$  or  $\text{K}^{\oplus}$ ) or an ammonium cation ( $\text{NH}_4^{\oplus}$ ).  $\text{A}_1\ominus$  is a monovalent anion, for example  $\text{Br}^{\ominus}$ ,  $\text{Cl}^{\ominus}$ ,  $\text{CH}_3\text{OSO}_3^{\ominus}$  or



The radicals W in the compounds of the formula (1) are groups which confer solubility in water; the number 40 of such radicals can be up to 4 ( $n=1$  to 4) and the preferred compounds contain 3, 2 or especially only one of the radicals W.

The compounds of the formula (2) contain a C=S grouping which is capable of tautomerism and can 45 therefore be described as follows.



For reasons of simplicity, in every case only one tautomeric form is indicated in the present specification, without, however, this excluding the other form.

A is a nitrogen atom



a carbon atom bonded via a double bond



grouping.

$\text{R}_2$  is hydrogen or also substituted or unsubstituted alkyl, for example having 1 to 10 carbon atoms and containing, for example, the substituents hydroxyl, amino, alkyl ( $\text{C}_1\text{C}_4$ ), halogen (fluorine, chlorine or bromine),  $-\text{SO}_3\text{M}$  or  $-\text{SO}_2\text{NH}_2$ ; furthermore,  $\text{R}_2$  can be substituted or unsubstituted phenyl, possible substituents being alkyl ( $\text{C}_1\text{C}_4$ ), halogen (fluorine, chlorine or bromine), hydroxyl, amino, carboxyl,  $-\text{SO}_3\text{H}$  or  $-\text{SO}_2\text{NH}_2$ ;  $\text{R}_1$  has the meaning defined for  $\text{R}_2$  with the exception of hydrogen; if  $\text{R}_1$  and  $\text{R}_2$  are the radicals of substituted (substituents as for phenyl) or unsubstituted, saturated or unsaturated 5-membered or 6-membered heterocyclic compounds containing nitrogen, oxygen and/or sulfur atoms, the radicals of heterocyclic compounds such as those mentioned under D can also be used here. If desired, the radicals  $\text{R}_1$  and  $\text{R}_2$  together can be the atom grouping which is still required to form a 4-membered, 5-membered or 6-membered heterocyclic ring with the grouping



25 Heteroatoms are the nitrogen, oxygen and/or sulfur atom.

E in the Bunte salts of the formula (3) has the meaning defined for D in the mercapto compounds of the formula (1) and D and E can be identical or different to one another. In addition, however, E can also be a bridge member of the formula  $-(\text{CH}_2)_{s-1}\text{CONH}(\text{CH}_2)_{t-1}-$ , in which s and t are each an integer from 1 to 3. Z has the meaning defined for W, and in this case also the two 30 symbols can have identical or different meanings.

35 B in the Bunte salts of the formula (3) is



The grouping  $-\text{E}-\text{B}-$  in  $-\text{E}-\text{B}-\text{SSO}_3\text{M}-$  ( $\text{r}=2$ ) can additionally be, for example, acetyl or benzoyl, which are unsubstituted or substituted by alkyl ( $\text{C}_1\text{C}_3$ ), preferably methyl, or halogen, preferably chlorine, for example:



60 The combination of (a) and (b) used in the process according to the invention is preferably a combination in which component (a) is a mercaptan of the formula



65 and component (b) is a Bunte salt of the formula



in which formulae  $D_1$  in each case is a substituted or unsubstituted aliphatic, araliphatic or aromatic radical having not more than 40 carbon atoms or a heterocyclic 5-membered or 6-membered ring which contains 1 to 4 nitrogen atoms, one oxygen atom and/or one sulfur atom and can be fused with a benzene ring,  $W_1$  is



$n_1$  and  $m_1$  in each case are an integer from 1 to 3 and  $M$ ,  $X$  and  $Y$  are as defined.

The symbols  $D_1$  in the formulae (4) and (5) can be 20 identical or different to one another.

Very suitable mercaptans of the formula (4) have the formula



in which  $D_2$  is an aliphatic or araliphatic radical having not more than 20 carbon atoms or a substituted or unsubstituted benzene radical and  $n_2$  is 1 or 2 and  $W_1$  is as 30 defined, and these mercaptans advantageously also have the formula



and are employed in combination with the Bunte salts of the formula



in which formulae  $D_2$  is as defined,  $W_2$  is  $-COOH$  or  $-SO_3M$ ,  $Z_2$  is  $-COOM$ ,  $-SO_3M$ ,  $-SSO_3M$ ,  $-NH_2$  or  $-OH$  and  $M$  is a monovalent cation and  $n_2$  and  $m_2$  are each 1 or 2.

The substituents on the benzene radical are, for example, alkyl having 1 to 4 carbon atoms, halogen (chlorine or bromine), hydroxyl, amino, carboxyl, sulfo ( $-SO_3H$ ) or sulfonamide ( $-SO_2NH_2$ ), and one or more of these substituents can be present.

The symbols  $D_2$  in the formulae (7) and (8) can be identical or different to one another.

If the mercaptans of the formula (7) contain an aromatic bridge member  $D_2$ , particularly preferred mercaptans are those of the formula



In this formula,  $D_3$  is phenylene, which can be unsubstituted or substituted by alkyl having 1 to 4 carbon atoms, halogen, especially chlorine, or amino ( $-NH_2$ ), whilst  $M$  is a monovalent cation, especially hydrogen ( $H^+$ ).

A particularly valuable combination of components 65 (a) and (b) which can be used in the process according to the invention contains, as component (a), a mercaptan of the formula



and, as component (b), a Bunte salt of the formula



in which formulae  $R_3$  is hydrogen, alkyl having 1 to 5 carbon atoms, carboxyl, carboxyalkyl having 1 to 3 carbon atoms in the alkyl moiety, phenyl, which is unsubstituted or substituted by alkyl having 1 to 4 carbon atoms, halogen, hydroxyl, amino,  $-SO_3H$ ,  $-COOH$  or  $-SO_2NH_2$ , or furyl, thienyl, pyrimidyl, pyridyl or 2-benzimidazolyl,  $R_4$  is hydrogen, alkyl having 1 to 5 carbon atoms, hydroxy- and mercapto-alkyl each having 1 to 3 carbon atoms, phenyl which is unsubstituted or substituted by alkyl having 1 to 4 carbon atoms, halogen, hydroxyl, amino,  $-SO_3H$  or  $-SO_2NH_2$ , or benzyl,  $R_5$  (if  $p$  is 1 or 2) is alkylene or alkylidene having not more than 6 carbon atoms, which is unsubstituted or substituted by alkyl having 1 to 4 carbon atoms, phenyl, halogen, hydroxyl, mercapto or amino, phenylene, which is unsubstituted or substituted by alkyl having 1 to 4 carbon atoms, halogen, hydroxyl, amino,  $-COOH$ ,  $-SO_3H$  or  $-SO_2NH_2$ , or  $\alpha,2-, \alpha,3-$  or  $\alpha,4$ -benzylene,  $R_{11}$  is hydrogen, alkyl having 1 to 5 carbon atoms, carboxyalkyl having 1 to 3 carbon atoms in the alkyl moiety, phenyl, which is unsubstituted or substituted by alkyl having 1 to 4 carbon atoms, halogen, hydroxyl, amino,  $-SO_3H$  or  $-SO_2NH_2$ , or benzyl, or also—if  $p$  is 1—a direct chemical bond.  $R_{12}$  (if  $q$  is 1 or 2) is alkylene or alkylidene having not more than 6 carbon atoms, which is unsubstituted or substituted by alkyl having 1 to 4 carbon atoms, phenyl, halogen, hydroxyl or amino, phenylene or aralkylene (benzylene or phenylethylene), which are unsubstituted or substituted by alkyl having 1 to 4 carbon atoms, halogen, hydroxyl, amino,  $-COOH$ ,  $-SO_3H$  or  $-SO_2NH_2$ ,  $-(CH_2)_{s-1}-CONH(CH_2)_{t-1}$  or—if  $q$  is 1—a direct chemical bond; if desired,  $R_{12}$  can also be acetyl or benzoyl, which are unsubstituted or substituted by alkyl having 1 to 3 carbon atoms or halogen;  $W_2$  is  $-COOM$  or  $-SO_3M$  and  $M$  is a monovalent cation;  $m_2$ ,  $p$  and  $q$  are each 1 or 2 and  $s$  and  $t$  are each an integer from 1 to 3.

Particularly preferred mercaptans of the formula (10) have the formulae



in which  $R_6$  is hydrogen, methyl, ethyl or phenyl,  $R_7$  is hydrogen, methyl, phenyl, tolyl or carboxymethyl,  $R_8$  is a direct chemical bond,



M is a monovalent cation and u is an integer from 1 to 3, and



in which R<sub>9</sub> and R<sub>10</sub> are each hydrogen, methyl or phenyl and u is an integer from 1 to 3, whilst particularly suitable Bunte salts are the compounds of the formulae



in which R<sub>13</sub> is hydrogen, methyl, ethyl, phenyl or carboxymethyl, R<sub>14</sub> is a direct chemical bond,



W<sub>2</sub> is —COOH or —SO<sub>3</sub>M, M is a monovalent cation and v is an integer from 1 to 6, and



in which R<sub>15</sub> is hydrogen, methyl or phenyl, M is a monovalent cation and w is 1 or 2.

The mercapto compounds and Bunte salts to be used according to the invention are compounds which are known per se and which are prepared by known methods. (cf., for example, R. Kerber, Tetr.Letters 1966, page 3,007, B. Milligan and J. Swan, Rev. pure and appl. chem. 12, 72 (1962) and H. Distler, Angew.Chem. 79, 520 (1967)).

A preferred process for the preparation of the sulfur compounds described above, and especially of the  $\beta$ -mercaptopcarboxylic acids and derivatives thereof, comprises introducing the —SH or —SSO<sub>3</sub>M groups into an  $\alpha,\beta$ -unsaturated carboxylic acid or derivatives thereof. Suitable reagents are, for example, hydrogen sulfide, thioacetic acid, carbon disulfide and derivatives thereof, thiourea and inorganic thiosulfates.

Suitable compounds for carrying out this process are, for example, the following unsaturated acids and their derivatives: acrylic acid, methacrylic acid, acrylonitrile, crotonic acid, 2- and 3-pentenoic acid, isopropylidenemalic acid, itaconic acid, maleic anhydride, crotononitrile, vinylacetic acid, citraconic acid, ethyl propiolate, mesaconic acid, allylacetic acid, 3,3-dimethylacrylic acid, tiglic acid, allylthioacetic acid, trans-aconitic acid, diethyl glutaconate, 2-hexenedioic acid dinitrile, allylmalonic acid, diethyl allylmalonate, 3-hexenedioic acid, 2-hexenoic acid, 3-cyclohexene-1-carboxylic acid, 6-heptenoic acid, cinnamic acid, methyl cinnamate, ethyl cinnamate,  $\alpha$ -methylcinnamic acid, 4-methylcinnamic acid, 2-, 3- or 4-methoxycinnamic acid, 4-hydroxycinnamic acid, 4-chlorocinnamic acid, 4-sulfamoylcinnamic acid, 3-hydroxy-4-methoxycinnamic acid, ethyl 4-sulfocinnamate, 2-carboxycinnamic acid, 3,4-methylene-dioxycinnamic acid, 2,3- or 3,4-dimethoxycinnamic acid, 3-(2'-furyl)-acrylic acid, 3-(2'-thienyl)-acrylic acid, 3-(3'-pyridyl)-acrylic acid, 3-(2'-pyridyl)-acrylic acid, 3-(4'-pyridyl)-acrylic acid, 5-norbornene-2-acrylic acid, 2-cyclopentenyl-1-acetic acid, 5-norbornene-2-carboxylic acid, bicyclo[2.2.2]oct-7-ene-2,3,5,7-tetracarboxylic acid anhydride, methyl 2-nonenoate, ethyl phenylpropionate, diethyl diallylmalonate, styrylacetic acid, 4-cyclooctene-1-carboxylic acid, 4-cycloheptene-1-carboxylic acid and 4,4'-diaminostilbene-3,3'-dicarboxylic acid. Furthermore, the acid halides of the said acids can also be employed. Furthermore, it is also possible to prepare Bunte salts by sulfonation of the corresponding mercaptans. Of course, other alkylating agents, especially 3-membered to 6-membered oxygen-heterocyclic compounds, for example epoxides, lactones or sultones, can also be employed for the preparation of the sulfur compounds to be used according to the invention.

| Examples of mercaptans                                                       | (Component a) |
|------------------------------------------------------------------------------|---------------|
| HOOC—CH <sub>2</sub> —SH                                                     |               |
|                                                                              |               |
| HOOC—CH <sub>2</sub> —CH <sub>2</sub> —SH                                    |               |
| HOOC—CH <sub>2</sub> —CH <sub>2</sub> —CH <sub>2</sub> —SH                   |               |
| HOOC—CH—CH <sub>2</sub> —SH                                                  |               |
|                                                                              |               |
| NH <sub>2</sub>                                                              |               |
| H <sub>2</sub> N—C—CH <sub>2</sub> —SH                                       |               |
|                                                                              |               |
| O                                                                            |               |
| HOOC <sub>2</sub> H <sub>4</sub> —NH—CO—CH <sub>2</sub> —CH <sub>2</sub> —SH |               |
|                                                                              |               |
| HO—CH <sub>2</sub> —CH—CH <sub>2</sub> —NH—CO—CH <sub>2</sub> —SH            |               |
|                                                                              |               |
| OH                                                                           |               |
| HOOC—CH <sub>2</sub> —NH—CO—CH <sub>2</sub> —SH                              |               |
|                                                                              |               |

-continued

## Examples of mercaptans

## (Component a)



-continued

-continued

## Examples of Bunte salts (Component b)



-continued

## Examples of Bunte salts (Component b)



$\text{M}$  = a monovalent cation, preferably the sodium, potassium or ammonium cation

- 40 The preferably aqueous developer solutions for developing a photographic material which has been exposed image-wise, which are to be used according to the invention, can in other respects have the compositions known per se.
- 45 For example, they contain dihydroxybenzenes, aminophenols, diaminobenzenes, pyrazolidinones, reductones or hydroxylamine derivatives as conventional compounds which develop silver halide.
- Conventional water-soluble silver halide solvents are,
- 50 for example, thioethers or thioamides, salts of thiocyanic acid, salts of sulfurous acid (sulfites) in high concentration and, preferably, salts of thiosulfuric acid (thiosulfates). The sulfites can, for example, as a rule be employed in an amount of more than 20 g/l, and if
- 55 desired also in smaller amounts, for example 10 to 20 g/l, and the thiocyanates and thiosulfates can be employed in a concentration of 0.1 to 200 g/l, in the aqueous preparations.
- The concentration of the thiosulfate is advantageously 10 to 200 g/l when used in a monobath and 0.1 to 10 g/l for masking developers for silver dye-bleach material. Suitable sulfur compounds are, in particular, those of the formulae (9) to (15). The sulfur compounds can also be used in developer preparations for reversal,
- 60 65 chromogenic, X-ray or black-and-white film materials.

Components (a) and (b) are preferably added to the aqueous developer preparation in amounts of 0.01 to 1 g/l and of 0.1 to 10 g/l respectively.

Thus, suitable developer solutions contain, for example, 0.1 to 20 g/l of the compound which develops silver halide, 0.1 to 200 g/l of the silver halide solvent and 0.05 to 10 g/l of the combination of components (a) and (b), the molar ratio of (a):(b) being 5:1 to 1:100 and preferably 1:1 to 1:20.

When preparing the aqueous developer preparations of the present invention it proves advantageous to mix in the combination of (a) and (b) some time before using the developer solution. The quantity ratio of Bunte salts to mercapto compounds can be varied within the indicated limits.

The developer solutions can be prepared, for example, from a single concentrate or from separate concentrates of the compound which develops silver halide, the silver halide solvent and the combination of components (a) and (b), and also, if desired, further components, by diluting with water, which can be mixed with organic solvents.

The concentrates can be in the form of a liquid or paste and if desired can also be in the solid form and, per liter of concentrate, can contain, for example, the individual components in 2 to 25 times the amount in which they are present in the ready-to-use developer solutions.

A very particularly valuable application of the present process comprises developing silver dye-bleach material, which has a layer build-up suitable for lowering the undesired secondary colour densities, with a developer preparation of the indicated composition.

Preferably, this relates to the process for the production of masked, subtractive, positive coloured images by the silver dye-bleach process, by exposure, silver developing, dye-bleaching, silver-bleaching and fixing and with the use of a photographic material which contains one image-wise bleachable dye in each of at least two layers, the absorption maximum of each dye corresponding to one of the three primary colours red, green

25

30

35

40

45

50

density which is to be compensated, there being at least a second dye, which has a main colour density which corresponds to a secondary colour density, of the first dye, which is to be compensated, and a silver halide emulsion which is free from iodide ions in a further layer and, moreover, a further layer, which is adjacent to that containing the second dye, containing colloidal nuclei which are capable of depositing metallic silver from soluble silver complexes and a septum being located between the layer containing the nuclei and the dye layer which has the secondary colour density which is to be compensated, and the silver developing bath with which the material is to be treated after exposure has taken place containing a ligand, which is able to produce water-soluble and diffusible silver complexes, as well as a combination of the compounds of the formulae (1) or (2) and (3). Particularly preferred combinations are those of compounds of the formulae (13) and (15).

The mixtures, to be used according to the invention, of mercapto compounds and Bunte salts are distinguished, inter alia, by the fact that they prevent the deposition of silver in developer solutions for an astonishingly long time. In contrast to the anti-sediment agents used hitherto, the mixtures of (a) and (b), which are used according to the invention, are otherwise photographically virtually inactive and very stable under the customary conditions, and this is advantageous in particular for a continuous procedure using the developers described.

In the examples which follow parts and percentages are by weight.

#### EXAMPLE 1

A photographic material for the silver dye-bleach process is prepared on a pigmented cellulose acetate base using the cyan image dye of the formula (101)



50

and blue and a silver halide emulsion layer sensitive in a specific spectral region being assigned to each dye, and

in the red-sensitised bottommost layer, the magenta dye of the formula (102)



65

a silver halide emulsion layer which at least partially consists of silver iodide being assigned, in this material, to the dye which has the undesired secondary colour

in a green-sensitised layer above this and the yellow dye of the formula (103)



in a blue-sensitive layer which is above the magenta layer.

The photographic material used is built up as follows (cf. German Offenlegungsschriften Nos. 2,036,918, 2,132,836 and 2,547,720):

Gelatin protective layer

Blue-sensitive, iodide-free AgBr emulsion

Yellow dye (103)+blue-sensitive, iodide-free AgBr emulsion

Yellow filter: yellow Ag hydrosol (40 mg/m<sup>2</sup>)

Green-sensitive AgBr/AgI emulsion

Magenta dye (102)+green-sensitive AgBr/AgI emulsion

Intermediate layer (gelatin)

Cyan dye (101)+red-sensitive AgBr/AgI emulsion

Red-sensitive AgBr/AgI Emulsion

Cellulose triacetate base, white opaque

Backing, gelatin

The layer build-up enables the blue secondary colour densities of the cyan dye and magenta dye to be corrected by additional bleaching of the yellow image dye as a function of the bleaching of the two other image dyes (blue-sensitive layer with yellow dye iodide-free; other dye layers with iodide-containing emulsion). The nuclei-containing layer is adjacent to the yellow dye layer. It additionally contains a yellow light filter dye and is separated from the magenta layer by a colourless emulsion layer (green-sensitive AgI-containing emulsion layer, which at the same time is the separating layer).

The iodide-containing emulsion layers contain crystals with 2.6 mol % of silver iodide and 97.4 mol % of silver bromide. The image dyes are used in a concentration such that their reflectance densities are each 2.0; the total silver content of the 22μ thick layers is 2.0 g/m<sup>2</sup>.

A coloured slide is copied on this material in an enlarger. The exposed material is processed in accordance with the following instructions (French Patent Specification No. 2,247,755). The processing temperature is 30° C.

1. Silver developing bath 3 minutes

|                                                      |                 |
|------------------------------------------------------|-----------------|
| tetrasodium salt of ethylenediamine-tetraacetic acid | 2 g/l           |
| 85% potassium hydroxide                              | 30 g/l          |
| boric acid                                           | 16 g/l          |
| potassium metabisulfite                              | 26 g/l          |
| 1-phenyl-3-pyrazolidinone                            | 0.35 g/l        |
| hydroquinone                                         | 5 g/l           |
| benztriazole                                         | 0.8 g/l         |
| potassium bromide                                    | 2 g/l           |
| anhydrous sodium thiosulfate                         | 0.8 g/l         |
| compound of the formula (104)                        | 0.5 g/l         |
| compound of the formula (105)                        | 0.85 g/l        |
|                                                      | (component (a)) |



-continued

|                                |           |  |
|--------------------------------|-----------|--|
| 2. Washing                     | 1 minute  |  |
| 3. Bleaching bath              | 5 minutes |  |
| 15 sulfamic acid               | 100 g/l   |  |
| sodium m-nitrobenzenesulfonate | 10 g/l    |  |
| 1-thioglycerol                 | 1 ml/l    |  |
| potassium iodide               | 6 g/l     |  |
| 2,3,6-trimethylquinoxaline     | 2 g/l     |  |
| 4. Washing                     | 1 minute  |  |
| 5. Fixing bath                 | 4 minutes |  |
| 20 ammonium thiosulfate        | 250 g/l   |  |
| potassium metabisulfite        | 50 g/l    |  |
| 85% potassium hydroxide        | 20 g/l    |  |
| 6. Washing                     | 6 minutes |  |

25 Total processing time 20 minutes

The reflection print of the slide which is obtained after drying is distinguished by faithful reproduction of the tonalities and by unadulterated colour reproduction.

As a result of the addition of the two compounds (formula (104) and formula (105)), the developer is usable for a relatively long time. Even after processing several colour enlargements, the solution remains clear, i.e. free from the deposition of metallic silver.

If only the compound of the formula (104) is added to the developer, the solution does indeed remain clear for a relatively long time, but the developer characteristics are changed: in the developed colour printing material, the yellow gradation in the shadows is too flat; the gradation equilibrium is thus disturbed. Colour prints processed with this developer have fewer saturated yellow tones. Moreover, darker parts of the image appear bluish-tinged.

If the developer contains only the compound of the formula (105), the solution becomes decolorised a short time after it is used; metallic silver separates out.

In place of the combination of the compounds of the formulae (104) and (105), it is also possible to employ other combinations of mercaptans and Bunte salts from the tables given above.

50

EXAMPLE 2

Material for the silver dye-bleach process is processed in accordance with Example 1 but the compounds of the formulae

|    |       |         |
|----|-------|---------|
| 55 | (106) | 0.5 g/l |
|    | (107) | 1 g/l   |

are used in the silver developing bath.

The developing time is 2 minutes at a temperature of 30° C. After drying, reflection prints of good image quality are obtained. Even when the developer is used repeatedly (total of 0.1 m<sup>2</sup> of material per liter of solution), no change in the image quality and no turbidity in the solution are to be found.

## EXAMPLE 3

A black-and-white developer of the following composition is prepared:

|                                                 |         |
|-------------------------------------------------|---------|
| potassium carbonate                             | 30 g    |
| sodium sulfite                                  | 100 g   |
| potassium bromide                               | 3 g     |
| hydroquinone                                    | 40 g    |
| ethylenediaminetetraacetic acid (disodium salt) | 1.5 g   |
| potassium hydroxide                             | 17 g    |
| water to make up to                             | 1 liter |

The solution is divided into two 500 ml portions A and B.

0.5 g of the compound of the formula (104) is added to portion A.

0.5 g of 2-aminoethane-thiolsulfonic acid and 0.5 g of the compound of the formula (104) are added to portion B.

Black-and-white camera films are developed with these solutions. Portion A remains clear for a certain time but turbidity due to a silver sediment can then be observed. The developer characteristics of this solution change in the manner indicated in Example 1.

Portion B, on the other hand, remains clear and retains its good developer characteristics even after prolonged use.

## EXAMPLE 4

A black-and-white developer of the following composition

|                             |         |
|-----------------------------|---------|
| 4-methylaminophenol-sulfate | 2 g     |
| hydroquinone                | 5 g     |
| sodium sulfite (anhydrous)  | 100 g   |
| borax                       | 3 g     |
| water to make up to         | 1 liter |

is mixed with 0.5 g of the compound of the formula (104) and 0.85 g of the compound of the formula (105).

Black-and-white camera films are each developed for 6 minutes at 20° C. with this solution in a tank. After a total of 10 36 exposure, size 135 films have been developed, the solution starts to become exhausted and must either be regenerated or replaced by fresh solution. In contrast to a developer solution which has been prepared without the addition of the compounds of the formulae (104) and (105), there is still no trace of the formation of silver sediment at this time.

What is claimed is:

1. A process for the prevention of darkening and the formation of a sediment in photographic developer solutions which contain a compound which develops silver halide, a water-soluble silver halide solvent and organic sulfur compounds, which comprises adding to the developer solution, as organic sulfur compounds, a combination of (a) a compound of the formulae



and (b) a Bunte salt of the formula



in which formulae A is a nitrogen atom, a carbon atom bonded via a double bond

5  $(=\text{C}-)$  or  $\text{CH}$  and B is  $\text{C}=\text{O}$  or  $\text{CH}_2\text{C}=\text{O}$ ,  
10 R<sub>2</sub> is hydrogen, substituted or unsubstituted alkyl, substituted or unsubstituted phenyl or a substituted or unsubstituted, saturated or unsaturated 5-membered or 6-membered heterocyclic radical containing nitrogen, oxygen and/or sulfur atoms and R<sub>1</sub> has the meaning defined for R<sub>2</sub> with the exception of hydrogen, or R<sub>1</sub> and R<sub>2</sub> together with the atoms to which they are bonded form a 4-membered, 5-membered or 6-membered heterocyclic ring, D and E are each a substituted or unsubstituted aliphatic, araliphatic, cycloaliphatic, aromatic or heterocyclic radical and W and Z are each a radical of the formulae



30 or a polyoxyethylene radical which has 2 to 20 oxyethylene units and can be sulfonated, in which formulae G, X and Y are each hydrogen or are alkyl having 1 to 6 carbon atoms which is substituted by hydroxyl, carboxyl or  $\text{---SO}_3\text{H}$  and Y is also phenyl, phenylsulfonic acid, alkylsulfonyl having 1 to 5 carbon atoms, phenylsulfonyl or tolylsulfonyl, and A<sub>1</sub><sup>⊖</sup> is a monovalent anion and M is a monovalent cation, and n and m are each an integer from 1 to 4 and r is 1 or 2.

40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920

-continued



$n_1$  and  $m_1$  in each case are an integer from 1 to 3 and M, X and Y are as defined in claim 1.

4. A process according to claim 3, wherein component (a) is a mercaptan of the formula



in which  $\text{D}_2$  is an aliphatic or araliphatic radical having not more than 20 carbon atoms or a substituted or unsubstituted benzene radical and  $n_2$  is 1 or 2 and  $\text{W}_1$  is as defined in claim 3.

5. A process according to claim 4, wherein component (a) is a mercaptan of the formula



and component (b) is a Bunte salt of the formula



in which formulae  $\text{D}_2$  in each case is an aliphatic or araliphatic radical having not more than 20 carbon atoms or a substituted or unsubstituted benzene radical,  $\text{W}_2$  is  $-\text{COOH}$  or  $-\text{SO}_3\text{M}$ ,  $\text{Z}_2$  is  $-\text{COOM}$ ,  $-\text{SO}_3\text{M}$ ,  $-\text{SSO}_3\text{M}$ ,  $-\text{NH}_2$  or  $-\text{OH}$  and M is a monovalent cation and  $n_2$  and  $m_2$  are each 1 or 2.

6. A process according to claim 5, wherein component (a) is a mercaptan of the formula  $\text{HS}-\text{D}_3-\text{COOM}$ , in which  $\text{D}_3$  is phenylene which is unsubstituted or substituted by alkyl having 1 to 4 carbon atoms, halogen or amino and M is a monovalent cation.

7. A process according to claim 6, wherein  $\text{D}_2$  is a straight-chain or branched alkylene having 1 to 10 carbon atoms, which is optionally interrupted by  $-\text{O}-$ ,  $-\text{SO}_2-$ ,  $-\text{NH}-$  or  $-\text{NR}-$ , in which R is alkyl having 1 to 4 carbon atoms.

8. A process according to claim 5, wherein component (a) is a mercaptan of the formula



and component (b) is a Bunte salt of the formula



in which formulae  $\text{R}_3$  is hydrogen, alkyl having 1 to 5 carbon atoms, carboxyl, carboxyalkyl having 1 to 3 carbon atoms in the alkyl moiety, phenyl, which is unsubstituted or substituted by alkyl having 1 to 4 carbon atoms, halogen, hydroxyl, amino,  $-\text{SO}_3\text{H}$ ,  $-\text{COOH}$  or  $-\text{SO}_2\text{NH}_2$ , or furyl, thienyl, pyrimidyl, pyridyl or 2-benzimidazolyl,  $\text{R}_4$  is hydrogen, alkyl having 1 to 5 carbon atoms, hydroxy- and mercapto-alkyl each having 1 to 3 carbon atoms, phenyl which is unsubstituted or substituted by alkyl having 1 to 4 carbon atoms,

halogen, hydroxyl, amino,  $-\text{SO}_3\text{H}$  or  $-\text{SO}_2\text{NH}_2$ , or benzyl,  $\text{R}_5$  is alkylene or alkylidene having not more than 6 carbon atoms, which is unsubstituted or substituted by alkyl having 1 to 4 carbon atoms, phenyl, halogen, hydroxyl, mercapto or amino, phenylene, which is unsubstituted or substituted by alkyl having 1 to 4 carbon atoms, halogen, hydroxyl, amino,  $-\text{COOH}$ ,  $-\text{SO}_3\text{H}$  or  $-\text{SO}_2\text{NH}_2$ , or  $\alpha,2-$ ,  $\alpha,3-$  or  $\alpha,4$ -benzylene or—if p is 1—a direct chemical bond,  $\text{R}_{11}$  is hydrogen, alkyl having 1 to 5 carbon atoms, carboxyalkyl having 1 to 3 carbon atoms in the alkyl moiety, phenyl, which is unsubstituted or substituted by alkyl having 1 to 4 carbon atoms, halogen, hydroxyl, amino,  $-\text{SO}_3\text{H}$  or  $-\text{SO}_2\text{NH}_2$ , or benzyl,  $\text{R}_{12}$  is alkylene or alkylidene having not more than 6 carbon atoms, which is unsubstituted or substituted by alkyl having 1 to 4 carbon atoms, phenyl, halogen, hydroxyl or amino, phenylene or aralkylene, which are unsubstituted or substituted by alkyl having 1 to 4 carbon atoms, halogen, hydroxyl, amino,  $-\text{COOH}$ ,  $-\text{SO}_3\text{H}$  or  $-\text{SO}_2\text{NH}_2$  or  $-(\text{CH}_2)_{s-1}-\text{CONH}(\text{CH}_2)_{t-1}$  or—if q is 1—a direct chemical bond,  $\text{Z}_2$  is  $-\text{COOM}$ ,  $-\text{SO}_3\text{M}$ ,  $-\text{SSO}_3\text{M}$ ,  $-\text{NH}_2$  or  $-\text{OH}$ ,  $\text{W}_2$  is  $-\text{COOM}$  or  $-\text{SO}_3\text{M}$ , M is a monovalent cation and  $m_2$ , p and q are each 1 or 2 and s and t are each an integer from 1 to 3.

9. A process according to claim 8, wherein component (a) is a mercaptan of the formula



in which  $\text{R}_6$  is hydrogen, methyl, ethyl or phenyl,  $\text{R}_7$  is hydrogen, methyl, phenyl, tolyl or carboxymethyl,  $\text{R}_8$  is a direct chemical bond,



M is a monovalent cation and u is an integer from 1 to 3.

10. A process according to claim 9, wherein component (a) is a mercaptan of the formula



in which  $\text{R}_9$  and  $\text{R}_{10}$  are each hydrogen, methyl or phenyl and u is an integer from 1 to 3.

11. A process according to claim 8, wherein component (b) is a Bunte salt of the formula



in which  $\text{R}_{13}$  is hydrogen, methyl, ethyl, phenyl or carboxymethyl,  $\text{R}_{14}$  is a direct chemical bond,



-continued



$\text{M}$  is a monovalent cation and  $v$  is an integer from 1 to 6.

12. A process according to claim 11, wherein component (b) is a Bunte salt of the formula



in which  $\text{R}_{15}$  is hydrogen, methyl or phenyl,  $\text{M}$  is a monovalent cation,  $\text{Z}_3$  is  $-\text{COOH}$  or  $-\text{NH}_2$  and  $w$  is 1 or 2.

13. A process according to claim 8, wherein component (a) is a mercaptan of the formula



and component (b) is a Bunte salt of the formula



in which formulae  $\text{R}_9$ ,  $\text{R}_{10}$  and  $\text{R}_{15}$  are each hydrogen, methyl or phenyl,  $\text{M}$  is a monovalent cation,  $u$  is an integer from 1 to 3 and  $w$  is 1 or 2.

14. A process according to claim 1, wherein the developer solution contains, as the silver halide solvent, a sulfite in a concentration of more than 20 g per liter or a water-soluble thiocyanate or thiosulfate.

15. A developer solution, for developing photographic recording material which contains silver halide and has been exposed image-wise, which contains a compound which develops silver halide, a water-soluble silver halide solvent and organic sulfur compounds, wherein the developer solution contains, as the organic sulfur compounds, a combination of (a) a compound of the formulae



and (b) a Bunte salt of the formula



in which formulae  $\text{A}$  is a nitrogen atom, a carbon atom bonded via a double bond



$\text{R}_2$  is hydrogen, substituted or unsubstituted alkyl, substituted or unsubstituted phenyl or a substituted or unsubstituted, saturated or unsaturated 5-membered or 6-membered heterocyclic radical containing nitrogen, oxygen and/or sulfur atoms and  $\text{R}_1$  has the meaning defined for  $\text{R}_2$  with the exception of hydrogen, or  $\text{R}_1$  and  $\text{R}_2$  together with the atoms to which they are bonded form a 4-membered, 5-membered or 6-membered heterocyclic ring,  $\text{D}$  and  $\text{E}$  are each a substituted or unsubstituted aliphatic, araliphatic, cycloaliphatic, aromatic or heterocyclic radical and  $\text{W}$  and  $\text{Z}$  are each a radical of the formulae



or a polyoxyethylene radical which has 2 to 20 oxyethylene units and can be sulfonated, in which formulae  $\text{G}$ ,  $\text{X}$  and  $\text{Y}$  are each hydrogen or are alkyl having 1 to 6 carbon atoms which is substituted by hydroxyl, carboxyl or  $-\text{SO}_3\text{H}$  and  $\text{Y}$  is also phenyl, phenylsulfonic acid, alkylsulfonyl having 1 to 5 carbon atoms, phenylsulfonyl or tolylsulfonyl, and  $\text{A}_1\text{---}$  is a monovalent anion and  $\text{M}$  is a monovalent cation, and  $n$  and  $m$  are each an integer from 1 to 4 and  $r$  is 1 or 2.

16. A developer solution according to claim 15 which is aqueous.

17. A developer solution according to claims 15 or 16, which contains 0.1 to 20 g/l of the compound which develops silver halide, 0.1 to 200 g/l of the silver halide solvent and 0.05 to 10 g/l of the combination of components (a) and (b), the molar ratio of (a):(b) being 5:1 to 1:100.

18. A developer solution according to claim 15 which is prepared from a single liquid or pasty concentrate of the silver halide developer, the silver halide solvent, the combination of components (a) and (b) and optionally further components by diluting with water or water/organic solvent mixtures, the amounts of the components being 0.2 to 500 g/l of the silver halide developer, 0.2 to 500 g/l of the silver halide solvent and 0.1 to 250 g/l of the combination of the components (a) and (b), the molar ratio of (a):(b) being 5:1 to 1:100.

19. A developer solution according to claim 15 which is prepared from separate liquid or pasty concentrates of the silver halide developer, the silver halide solvent, the combination of components (a) and (b) and optionally further components by diluting with water or water/organic solvent mixtures, the amount of the components being 0.2 to 500 g/l of the silver halide developer, 0.2 to 500 g/l of the silver halide solvent and 0.1 to 250 g/l of the combination of the components (a) and (b), the molar ratio of (a):(b) being 5:1 to 1:100.

20. A concentrate for the preparation of a developer solution according to claim 1 which contains 0.2 to 500 g/l of the silver halide developer, 0.2 to 500 g/l of the silver halide solvent, 0.1 to 250 g/l of the combination of the components (a) and (b), the molar ratio (a):(b)

being 5:1 to 1:100, and optionally further components, and being in a form of a liquid or a paste.

21. A liquid or pasty concentrate according to claim 20, which contains the individual components, per liter of concentrate, in amounts which are 2 to 25 times the following amounts: 0.1 to 20 g/l of the compound

which develops silver halide, 0.1 to 200 g/l of the silver halide solvent and 0.05 to 10 g/l of the combination of components (a) and (b), the molar ratio of (a):(b) being 5:1 to 1:100.

\* \* \* \* \*

10

15

20

25

30

35

40

45

50

55

60

65